# EUROPEAN PATENT SPECIFICATION

(11) **EP 2 225 399 B1**
(45) Date of publication and mention of the grant of the patent: **20.11.2013**
(21) Application number: 08865001.5
(22) Date of filing: 09.12.2008
(51) Int. Cl.: C14C 9/02, C14C 3/28

(54) **RETANNING AND FATLIQUORING AGENT FOR LEATHER**
NACHGERBMITTEL UND FETTLICKER FÜR LEDER
AGENT DE RETANNAGE ET LIQUEUR GRASSE POUR CUIR

(30) Priority: 19.12.2007 EP 07024581
(43) Date of publication of application: 08.09.2010
(73) Proprietor: Clariant Finance (BVI) Limited, Road Town, Tortola (VG)
(72) Inventor: GAMARINO, Roberta, I-15033 Casale Monferrato (IT); TRIMARCO, Licia, I-21047 Saronno (IT); GIANI, Michele, I-21052 Busto Arsizio (IT); REINEKING, Claus, 71111 Waldenbuch (DE)
(74) Representative: Mikulecky, Klaus
(86) International application number: PCT/EP2008/067062
(87) International publication number: WO 2009/080489

(56) References cited:
- DE-A1- 4 402 029
- US-A- 5 279 613
- US-A- 5 554 306
- US-A- 5 575 939

## Description

The invention relates to a composition for wet retanning and fatliquoring of pelts, skins, hides, leather intermediate products or non-finished leather and to its production and use.

For wet retanning and fatliquoring the leather industry is using different compounds, especially polymeric compounds have been proposed for obtaining soft and firm leather types.

US 5,279,613 discloses copolymers which are obtainable by free radical copolymerization of (a) C₈-C₄₀-monoolefins with (b) ethylenically unsaturated C₄-C₈-dicarboxylic anhydrides by mass polymerization at from 80°C to 300°C to give copolymers having molecular weights of from 500 to 20,000 g/mol, subsequent solvolysis of the anhydride groups of the copolymers and partial or complete neutralization of the carboxyl groups formed during the solvolysis, in an aqueous medium by means of a base, and which are present in the form of aqueous dispersions or solutions, which are used as agents for rendering leathers and skins water-repellent.

US 5,575,939 discloses a process for the fat liquoring/softening of leathers and furs by treatment with an aqueous dispersion of a copolymer obtainable by polymerization of a) maleic anhydride, b) C₁₂-C₃₀ alpha-olefins, esters of (meth)acrylic acid and/or maleic acid with C₁₂-C₃₀ alcohols and c) optionally, further hydrophilic, ethylenically unsaturated monomers which are copolymerizable with a) and b), reaction of the anhydride groups with monovalent alcohols comprising at least one ether functionality, and partial neutralization or hydrolysis of the residual acid or anhydride groups and manufacture of a flowable dispersion having an active substance content of at least 40%-wt.

Nevertheless there is always a need for compounds with even better properties.

It has now surprisingly been found that with the below defined composition, there can be achieved in wet retanning and fatliquoring of pelts, skins, hides, leather intermediate products or non-finished leather an outstanding and highly satisfactory retanning and fatliquoring of the substrates.

Therefore an object of the instant invention is a composition consisting of the components (A), (B) and (C) wherein:
(A) is a reaction product of an ethylenically unsaturated C₄-C₈-dicarboxylic anhydride with C₃-C₄₀-alpha-olefins, used in acid form or preferably followed by partial or total neutralisation with a base in aqueous dispersion with or without solvents, optionally part of the anhydride groups are reacted with alcohols, polyalcohols, glycols or organic amines,
(B) is a reaction product of ethylenically unsaturated C₄-C₈-dicarboxylic anhydrides with C₁₀-C₄₀-fatty acids or C₄-C₃₀ polycarboxylic acids or C₁₀-C₄₀ fatty alcohols or oxo-alcohols or glycols or polyglycols or C₃-C₂₀ organic amines, all being saturated or unsaturated, linear or branched and the fatty acids being ethoxylated and/or propoxylated or having been reacted with polyglycols or glycols, and the polycarboxylic acids being ethoxylated and/or propoxylated or having been reacted with polyglycols or glycols at least with one carboxylic group, whereas the fatty alcohols or oxo-alcohols and the fatty amines can optionally be ethoxylated and/or propoxylated, and
(C) is a reaction product of (B) with bisulphite or metabisulphite or sulphite or sulphuric acid or oleum preferably neutralised with a base where the base is an alkali or earth alkali hydroxide, ammonia or an organic amine in aqueous dispersion with or without solvents.

In the component (B) the glycols or polyglycols can be reacted with other carboxylic acids or C₄-C₃₀ polycarboxylic acids or derivates of carboxylic or polycarboxylic acids.

This composition provides excellent softening and retanning properties which can make further treatment with retanning and lubricating agents unnecessary. It confers outstanding chemical and physical properties to the leathers: excellent fogging values, good light and heat stability, no spue problems, ecological advantage: low COD in the bath, no phenol or formaldehyde in the bath as well as in the leather (usually present in bath and leather after treatments with common retanning agents), properties which otherwise are very difficult to reach with the standard fatliquoring and retanning agents already available on the market.

Preferred are compositions wherein
in the component (A) the dicarboxylic anhydride is maleic anhydride and the alpha-olefins have a chain length of 12 to 30 C-atoms and the base is ammonia, an amine or an alkali or earth alkali hydroxide in aqueous dispersion with or without solvents,
in the component (B) the dicarboxylic anhydride is maleic anhydride, and the fatty acids or fatty alcohols or oxo-alcohols have a chain length of 12 to 30 C-atoms and are ethoxylated/propoxylated with 2- 25 mol of EO/PO (ethylene oxide/propylene oxide) or the fatty acids are reacted with polyglycols 100 - 1200,
the component (C) is a reaction product of (B) with sodium bisulphite carried out in aqueous dispersion.

Especially good properties show compositions wherein
in the component (A) the alpha-olefins have a chain length of 18 to 24 C-atoms and the base is NaOH,
in the component (B) the fatty acids or fatty alcohols or oxo-alcohols have a chain length of 12 to 20 C-atoms and have one or more double bonds, and the fatty acids and fatty alcohols or oxo-alcohols have been ethoxylated and optionally the fatty acids have been reacted prior to the reaction with maleic anhydride with polyethylene glycols or glycols.

Examples of said fatty acids used for (B) are lauroleic acid, miristoleic acid, palmitoleic acid, oleic acid, linoleic acid, or alpha-linolenic acid. Preferred are oleic acid and linoleic acid or mixtures thereof, and especially preferred is oleic acid.

Preferred examples of said alcohols used for (B) are oleyl alcohol, linoleyl alcohol, cetyloleylalcohols or mixtures thereof as well as branched alcohols from oxo-synthesis like C₉, C₁₀, C₁₁, C₁₂, C₁₃ - C₁₄, C₁₅ oxo-alcohols or mixtures thereof.

Especially preferred compositions are those wherein
in the component (A) the alpha-olefins have a chain length of 20 to 22 C-atoms,
in the component (B) the fatty acid is oleic acid and wherein the polyethylene glycol is a polyethylene glycol of the formula HO(CH₂CH₂O)ₙH with an average number of n from 2 to 25 (like for example "polyglycol 100 - 1200").

The alpha-olefins used are commercial products. A chain length of 20 to 22 C-atoms does not exclude smaller amounts (up to 10 mol-%) of C₁₈ or shorter and C₂₄ or longer.

The oleic acid used is a commercial product from natural sources , that means mixture of fatty acids C₁₂-C₁₈ whereas the percentage of oleic acid is > 60%.

The instant compositions in general have a molar ratio of (A):[(B) + (C)] of from 5:100 to 100:5 and a molar ratio of (B):(C) of from 5:100 to 100:5.

Preferred are compositions wherein the molar ratio of (A):[(B) + (C)] is from 50:100 to 100:50, more preferably from 70:100 to 100:70 and the molar ratio from (B):(C) is from 20:100 to 100:20, more preferably from 60:100 to 100:60.

The instant compositions may further comprise amides and esters of (A) as described in US 5,279,613. Details of these amidation and esterification reactions are found in this prior art.

The instant compositions may further comprise at least one formulation additive (S) e.g. for adjusting the physical aspect of the composition and/or its use properties and may be selected from water or an organic solvent or a solubiliser or mixtures thereof, said additives being miscible with or soluble in (A) and (B) and (C) or in which (A) and (B) and (C) are soluble. Furthermore at least one of the following additives or mixtures thereof may be contained: defoamers, natural or mineral oils, surfactants, lecithines, biocides.

(S) may in particular comprise one or more solvents and/or solubilisers and/or a defoamer and/or one or more surfactants and/or mineral or natural oil and/or a biocide. Preferably (S) is selected from the group comprising (S1) water, (S2) an organic solvent or mixture of organic solvents and/or a solubiliser or mixture of solubilisers, miscible with or soluble in (A) and (B) and (C) or in which (A) and (B) and (C) are soluble, (S3) a defoamer and/or (S4) a surfactant and/ or (S5) a mineral or natural oil and/or (S6) synthetic or natural lecithine and/ or (S7) a biocide.

Preferably (S2) is an organic solvent miscible with water, which is aliphatic and contains at least one oxygen and no other heteroatoms, or a mixture of two or more of such solvents. More preferably (S2) is selected from the group consisting of aliphatic mono- or oligofunctional alcohols and mono- or di-(C₁-C₄-alkyl)-ethers thereof. (S2) may include water-miscible, saturated aliphatic solvents of ether and/or alcohol character. As (S2) there may in particular be employed a C₃-C₄-alkanol, a diol which is a C₂-C₄-alkylene glycol or a higher diol e.g. with 6 carbon atoms mainly 2-methyl-2,4-pentanediol (hexylene glycol), dipropylene glycol or a di-. tri- or tetraethylene glycol, and mono- or di-(C₁-C₄-alkyl)-ethers thereof, or glycerol. Particularly preferred solvents or solubilisers (S2) include e.g.: isopropanol, mono- or dipropylene glycol, mono-, di-, tri- or tetraethylene glycol, hexylene glycol, mono- or dipropylene glycol monomethylether, ethylene glycol monobutylether and methyl, ethyl, isopropyl or butyl mono- or diethers of di-, tri- or tetraethylene glycol.

As solvents/solubilisers in (S) there may be employed water (S1) alone, solvent or solubiliser (S2) alone or a mixture of water (S1) and solvent or solubiliser (S2).

As defoamers (S3) there may be employed known products in the commercially available forms, like, for example, silicones, silica, paraffins, paraffin oil, mineral oil or trialkylphosphates (e.g. triisopropyl-phosphate or tributylphosphate), ethers, alkoxylated fatty esters, alkoxylated fatty acids, in an efficient concentration, e.g. below 0.2 % by weight, preferably below 0.1% by weight, referred to the dry content of (A)+(B)+(C). Mostly a defoamer (S3) is not necessary and is not added.

As surfactants (S4) there may be employed any conventional non ionic or anionic surfactants in particular with emulsifier character.

As non ionic surfactants are preferably employed alkoxylated, mainly ethoxylated, alcohols. As alkoxylated alcohols can also be employed some alkoxylated, preferably ethoxylated oxo-alcohols.

As anionic surfactant preferably emulsifiers contain a sulpho group, optionally a phosphorus group. Preferably as anionic surfctant (S4) are employed arilaliphatic or more preferably aliphatic sulphates, which may contain a heteroatomic bridge in the aliphatic chain (e.g. an ester, amine, amide or preferably ether bridge) and which contain a lipophilic hydrocarbon radical e.g. with 7 to 24 carbon atoms, more preferably sulphuric acid monoesters of fatty alcohols or of ethoxylated (e.g. mono- to oligo-ethoxylated) fatty alcohols or fatty amine with e.g. 12 to 24 carbon atoms in the fatty hydrocarbon radical. Among these the sulphuric acid esters of ethoxylated fatty alcohols are preferred. Optionally as anionic surfactant are employed arilaliphatic or more preferably aliphatic mono- or di-phosphoric acid esters or mixture thereof. Among these the phosphoric acid esters of ethoxylated fatty alcohols are preferred.

The anionic surfactants (S4) are preferably in the form of alkali metal salts, more preferably sodium or potassium salts.

As mineral or natural oils (S5) may be employed hydrocarbons fluid got by distillation of the oil, paraffinic hydrocarbons and / or natural or synthetic waxes or vegetable or animal tryglycerides.

If desired to modify the applicative properties may be employed synthetic or natural lecithine (S6). Mostly the lecithine is not necessary and is not added.

As biocide (S7) there may be employed known products in the commercially available forms, e.g biocide based on 1,2-benzoisotiazolin-3-one and 1,2-dibromo-2,4-dicianobutano, biocide based on chloro or chloro free isotiazolinoni, based on bronopol, based on 2-(tiocianometiltio)-benzotiazolo or based on p-cloro-m- cresol. These products can be employed alone or in mixture.

The polymers (A) are basically known products and are for example described in US 5,279,613, US 5,575,939 or DE 3 730 885. Details of their preparation are also disclosed in these documents.

The instant compound (B) is not a polymerization product where a radical polymerization takes place and therefore still contains double bonds, in contrast to the product of US 5,575,939 where a radical polymerization takes place.

Component B can be obtained by heating the mentioned starting compounds at a temperature in the range 80 - 160 °C, with water distillation if required, optionally under vacuum for 2 - 6 hours and in the presence of an organic solvent, if necessary.

The ethoxylated products or ethoxylated and propoxylated products (fatty acids, fatty alcohols, oxo-alcohols) are known or may be produced in a manner conventional per se by addition reaction of ethylene oxide or of ethylene oxide and propylene oxide to the mixtures of fatty acids, fatty alcohols, oxo-alcohols, or organic amines.

As ethoxylation there is meant herein the addition reaction of ethylene oxide (also known as oxyethylation). As propoxylation there is meant herein the addition reaction of propylene oxide (also known as oxypropylation).

The addition reaction may be carried out under reaction conditions known per se, preferably in the presence of an alkali metal hydroxide, e.g. sodium hydroxide or potassium hydroxide, with heating, e.g. at a temperature in the range of 90 to 240°C, preferably 130 to 220°C in a closed vessel, in the presence of an inert gas, e.g. nitrogen. If propylene oxide is also reacted, it is preferably reacted first, followed by the reaction of ethylene oxide. Propylene oxide, if used, is employed in a minor proportion, preferably in this case there being added 1 to 2 moles of propylene oxide per mole of fatty acids or fatty alcohols or oxo-alcohols or organic amines mixture; more preferably no propylene oxide is added, but the mixture of fatty acids or fatty alcohols or oxo-alcohols or organic amines is reacted only with ethylene oxide. The molar proportion of ethylene oxide referred to fatty acids or fatty alcohols or oxo-alcohols or organic amines or mixtures thereof is in the range of 2 to 25, preferably 6 to 14.

The reaction of fatty acids with polyglycols can be carried out at a temperature in the range of 80-160°C for 2 - 6 hours optionally under vacuum (like for example 50-70 mm Hg), preferably with an acid catalyst like methansulfonic acid, as example.

Parts of component (B) are further reacted to synthesize (C) with sodium bisulphite at a temperature in the range of 60-120 °C for 2-10 hours in the presence of water, earth alkali hydroxides and, if necessary, organic solvents (like for example 2-propanol). The preferable pH range during the reaction is 5-8.

The compositions of the invention may be produced in a manner conventional per se, e.g. by mixing the components (A), (B) and (C) and any formulation additive (S).

The admixing of (A) with (B) and (C) and any (S) may be carried out e.g. at a temperature in the range of 15 to 70°C.

More preferably the corresponding mixture of (B) and (C) is prepared in a reactor with the required addition of sulphite or bisulphite or sulphuric acid or oleum agent to (B) and follows the neutralization with a base in the presence of water and, if necessary, organic solvents, and then (A) is added and (S) is added, if desired, at a temperature in the range of 15 to 70°C.

Of course, it is also possible to add the mixture of (B) and (C) to the component (A) that can already be added with (S), if desired, mixing all the components at a temperature in the range of 15 to 70°C.

It is also possible to add the mixture of (B) and (C) to the component (A) and then (S) is added, if desired, mixing all the components at a temperature in the range of 15 to 70°C.

The so produced compositions are ready for use. They are of satisfactory stability to storage and transportation. They are readily dilutable with water resulting in an aqueous dispersion and may e.g. be directly dosed into the treatment bath.

The aqueous dispersions thus obtainable are stable and have a long shelf life. They are very suitable for treating leathers and skins because they have a particularly pronounced action in fatliquoring and retanning. In many cases no additional fatliquoring agents based on natural or synthetic fatliquoring oils are required. The dispersions impart to the product good body and high tensile strength and tear strength, so that additional treatment with commercial retanning agents, for example with vegetable tanning agents or synthetic organic tanning agents (syntans) based on phenolsulfonic acid/phenol/formaldehyde condensates, is no longer necessary in most cases.

The dispersions described above are suitable for the treatment of all conventional tanned hides, in particular hides tanned with mineral tanning agents, such as chromium(III) salts.

The invention further provides a process for wet retanning and fatliquoring of tanned pelts, skins, hides, leather intermediate products or non-finished leather (crusted leather) or pelts, characterised in that a composition as defined above is employed as a retanning and fatliquoring agent.

In particular the invention provides a process for the production of leather, pelts or furskins, comprising in their production at least a wet degreasing treatment, a tannage, a retanning, a fatliquoring and a dyeing or finishing treatment, wherein retanning and fatliquoring can be carried out in one step with the instant composition or completed, if desired, with other commercial fatliquoring and retanning products.

As a substrate according to the invention there may be employed any hides, skins or pelts as conventionally processed in the beamhouse, tanned conventionally to get a wet blue or wet white leathers. There may e.g. be mentioned pelts, hides or skins from cow, sheep, goat, swine, cattle and other animals (e.g. horse, colt, reptiles - e.g. snake, lizards, water reptiles -, doe, deer, ostrich, poultry, dromedary, camel and camel-like animals - e.g. lama or alpaca -), and woolled skins (mainly from sheep or goat) and furskins.

Retanning and fatliquoring according to the invention may also be applied to leather intermediate products or non-finished leather (crusted leather). Thus if the substrate has already been tanned or retanned, the instant composition may be used before dyeing, mostly in order to improve dyeability e.g. uniform dispersion and distribution of the dye, or after dyeing to confer a fuller and deeper dyeing, or before finishing in order to prepare the substrate for a particular uniform link of the finishing.

To the retanning and fatliquoring bath there may e.g. be added one or more anionic surfactants (G) and/or a water miscible solvent (H).

As surfactants (G) of anionic character there may be employed any conventional surfactants, preferably those containing a sulpho group, e.g. aliphatic or arylaliphatic sulphates (G₁) or sulphonates (G₂), which may contain a heteroatomic bridge in the aliphatic chain (e.g. an ester, ether or preferably amide, bridge, an ether bridge being with particular preference part of a glycol ether chain) and which contain a lipophilic hydrocarbon radical e.g. with 7 to 24 carbon atoms. They are preferably in the form of alkali metal salts, more preferably sodium or potassium salts.

Suitable sulphates (G₁) are e.g.:
- (G₁'): sulphuric acid monoesters of fatty alcohols or of ethoxylated (e.g. mono-to oligo-ethoxylated) fatty alcohols or fatty amine with e.g. 12 to 24 carbon atoms in the fatty hydrocarbon radical,
- (G₁"): sulphuric acid esters of fatty acid monoglycerides with e.g. 12 to 24 carbon atoms in the fatty acid radical,
- (G₁"'): products of sulphation of unsaturated fatty acids or unsaturated oils (fatty acid triglycerides) with e.g. 18 to 22 carbon atoms in the unsaturated fatty acid radical or of ricinoleic acid or castor oil.

Suitable sulphonates (G₂) are e.g.
- (G₂'): fatty alkyl sulphonates and isothionates, with e.g. 12 to 24 carbon atoms in the fatty hydrocarbon radical, petroleum sulphonate (mainly secondary sulphonates with e.g. 10 to 15, usually 12 to 13, carbon atoms in the aliphatic chain),
- (G₂"): fatty acid taurides and N-methyltaurides with e.g. 12 to 24 carbon atoms in the fatty acid radical,
- (G₂'"): products of sulphitation of unsaturated fatty acids or unsaturated oils (fatty acid triglycerides) with e.g. 16 to 24 carbon atoms in the unsaturated fatty acid radical,
- (G₂""): mono- and di-alkyl-benzene sulphonates with e.g. a total of 1 to 12 carbon atoms in the alkyl substitution, e.g. with 4 to 12 carbon atoms in the alkyl chain, or short chain alkyl-benzene sulphonates with 1 to 3 carbon atoms in the alkyl radical and in the total alkyl substitution.

As mono- to oligo-ethoxylated in (G₁') there is meant the addition product of 1 to 10 moles of ethylene oxide to one mole of fatty alcohol. As examples of (G₁) there may be mentioned in particular lauryl sulphate, stearyl sulphate, and the sulphates of the addition product of 1 to 6 moles of ethylene oxide to one mole of lauryl or stearyl alcohol. As examples of (G₂) there may be mentioned in particular toluene-, xylene- or cumene-sulphonic acids, and fatty acid taurides or N-methyl taurides with on average 16 to 20 carbon atoms in the fatty acid radical. They are preferably in the form of potassium salts or more preferably sodium salts.

The solvents (H) are water-miscible, organic, preferably aliphatic solvents containing at least two linked oxygen atoms per molecule in the form of alcoholic hydroxy groups and/or ether bridges, and are in particular exempt of other heteroatoms than oxygen. There may in particular be mentioned saturated aliphatic compounds of ether and/or alcohol character, mainly mono-, di-, tri- and/or tetra-alkylene glycols and their mono-or di-(C₁₋₄-alkyl) ethers, preferably with ≥ 4 carbon atoms in the molecule, more preferably with ≥ 6 carbon atoms, e.g. butane-2,3- or -1,4-diol, dipropylene glycol, monomethyl ether of mono- or dipropylene glycol, and methyl-, ethyl-, isopropyl- or butyl-ethers of mono-, di-, or triethylene glycol, among which the monoalkylethers are preferred, especially diethylene glycol mono-butyl ether.

According to one feature of the invention one or more anionic surfactants (G) and/or a water miscible solvent (H) can be added to the instant composition.

Wet retanning and fatliquoring with the instant composition may be carried out analogously to methods known per se, expediently in a treatment drum or in a rotated aqueous bath e.g. in the range of 3 to 100 %, preferably 5 to 40 %, more preferably 5 to 15 % by weight referred to the wet shaved weight of the substrate for tanned leathers (wet blue leather or wet white leathers) and to the dry weight of the substrate for crusted leathers.

The temperature T of the retanning and fatliquoring bath advantageously is in the range of 20 to 60°C, preferably 30 to 60°C. The pH may be as desidered and advantageously is in the range 3,0 - 6,5 .

Retanning and fatliquoring may be carried out in one or more stages, and in each stage it may be carried out in one or more steps, preferably two, even if one is already sufficient to get a good penetration and an homogeneous dispersion of the agents. If it is carried out in two steps, one step may be regarded as the main step for the retanning and fatliquoring, while the second step may be regarded as a follow-up step for improving the effects and the substrate properties.

According to one feature of the invention, the instant composition may be used alone or if desired in the presence of one or more further retanning or other fatliquoring products expecially if leathers are manufactured to get particular articles, like automotive upholstery leathers.

According to one feature of the invention at least a part of said composition may be combined with other retanning or fatliquoring products. Preferably, however, any or at least the major required proportion of other retanning or fatliquoring agents are added separately to the bath, as desired and as suitable in the concerned treatment stage and/or step.

For retanning and fatliquoring of tanned substrates it is of advantage to use for the setting of bath and also for rinsing from 100-400 % of water and of an organic acid like formic acid, acetic acid etc., e.g. of a concentration in the scope from 0.1 to 5 %, preferably 0.1 to 0.5 % by weight and 0.2 - 3.0 % of a common wetting agent (a single component or a formulation) referred to the wet shaved weight of the substrate.

As wetting agent can be employed one or more anionic surfactants and one or more non ionic surfactants, preferably is employed one of more formulations of these surfactants present on the market for this scope.

Then the substrate is drained, the bath is added with water from 50 to 300 %, the pH is increased by addition of conventional bases or buffer salts such as sodium acetate, sodium formiate from 1.0 to 4.0 % or sodium bicarbonate from 0.5 to 3.0 % or other products having neutralising/buffering properties.

The bath is drained, again well washed with water from 50 to 400 % and drained again.

The retanning and fatliquoring treatment of the invention may be carried out for a duration as conventional per se for retanning and fatliquoring e.g. in the range of 1 to 4 hours, preferably 40 - 70 minutes for every treatment stage (in one or two steps).

For retanning and fatliquoring of crusted substrates it is of advantage to use for the setting of bath and also for rinsing from 200-800 % of water and of an organic acid like formic acid or acetic acid, e.g. of a concentration in the scope from 0.2 to 5 %, preferably 0.2 to 2.0 % by weight and 0.2 - 4.0 % of a wetting agent (alone or in formulation as many are available on the market) referred to the dry weight of the substrate.

As wetting agent can be employed one or more anionic surfactants and one or more non ionic surfactants, preferably is employed one of more formulations of these surfactants present on the market for this scope.

Then the substrate is drained, the bath is added with water from 100 to 600 % , the pH is increased by addition of conventional bases or buffer salts such as sodium acetate, sodium formiate from 2.0 to 8.0 % or sodium bicarbonate from 1.0 to 6.0 % or other products having neutralising/buffering properties.

The substrate is drained, again well washed with water from 100 to 800 % and drained again.

The retanning and fatliquoring treatment of the invention may be carried out for a duration as conventional per se for retanning and fatliquoring e.g. in the range of 1 to 4 hours, preferably 40 - 70 minutes for every treatment stage (in one or two steps).

After completion of the retanning and fatliquoring treatment, which preferably is followed by adjustments of pH or washing, the substrate may be directly further processed in the foreseen sequence of treatments for the production of the leather or pelt as desired. If desired, the retanning and fatliquoring substrates may even be washed, eventually added with biocides, drained and dried, for being e.g. stored or shipped in order to be further treated at a later stage. Preferably, however, the treatment sequence is not interrupted after retanning and fatliquoring, but the substrate is further treated in the same apparatus. The substrate retanned and fatliquored according to the invention is readily and optimally suitable for each of the subsequent treatments.

By the process of the invention there may be achieved an outstanding degree of retanning and fatliquoring of the substrate at once. In particular may be achieved a surprisingly good retanning and fatliquoring, without impairing other characteristic properties of the substrate, such as quality of the leather structure (especially the grain structure), handle, dyeability, light fastness, heat fastness, fogging of the finished leathers while a subsequent treatment with any chemicals finds in the substrate retanned and fatliquored according to the invention a substrate of high suitability for even distribution of the applied products, e.g., filling agents, other (re)tanning agents, dyestuffs, pigments, leather softeners, so that dyed and/or finished leathers and pelts of optimum quality are obtainable with a high yield of the corresponding applied products.

### EXAMPLES

The following examples shall explain the instant invention in more detail. If not indicated otherwise, parts and percentages are by weight and in the Application Examples the percentages refer to the wet shaved weight of the substrate, if not otherwise indicated. The starting materials employed in Examples and the additives employed in the Application Examples further to the retanning and fatliquoring agent, are commercially available products. The water used is a soft - middle hard water (max. 13-14 °F of hardness).

I.U.C. standards mentioned in the Application Examples are international standards in leather testing as recommended in IULTCS (International Union of Leather Technologists and Chemists Societies)

### PREPARATION EXAMPLES

### EXAMPLE 1

196 g of oleic acid are charged in a reactor and, under stirring, 139.0 g of polyglycol 200 are added and 1.3 g methan sulfonic acid are added. The mixture is heated up to 90-105 °C under vacuum (residual pressure of 50-70 mm Hg in reactor) and maintained at that temperature for 3-4 hours distillating water (water to be destilled: 12,5 g).

323,8 g. of reaction mass is cooled down to 80-90 °C and added with 34.1 g. of maleic anhydride. A weak exothermic reaction takes place. Then the reaction mass is heated up to 88 - 92 °C and kept at 88 - 92 °C for 30-40 minutes.

Then within 2-3 hours the temperature of the mass is increased to 100 - 110 °C under vacuum (residual pressure in reactor is 50-60 mmHg ): condensation water is destilled.

The reaction mass is then heated up to 120 - 130 °C and kept at 120 - 130 °C for 2-3 hours, destilling water. Amount of water to be destilled: 6,3 g. of water.

Yield of reaction: 351,6 g

### EXAMPLE 2

351,6 g of product prepared as indicated in example 1 are charged in reactor and heated to 80 - 90 °C and added with an aqueous solution of sodium metabisulphite and NaOH, prepared by mixing 88 parts of water with 33 parts of metabisulphite and 27.5 parts of NaOH sol. 30%.

The mixture is heated up to 85-98 °C for 2-3 hours.

### EXAMPLE 3

745 g of α-olefine are charged in a dry reactor and heated up to 148-152 °C. At 140-145°C 36 g of ditert-butylperoxide are added. Then during one hour, 275 g of maleic anhydride, melted at 80-90° C, are added under nitrogen flow and at a temperature of 150-165°C. When the addition is finished the mixture is heated three hours at 155-165°C. At the end of the reaction, the polymerization product is poured into an aqueous solution pre-heated at 80°C of 3200g of water and 475 g of sodium hydroxide 30% sol. The mixture is stirred one hour at 88-92°C and then cooled at 30-35°C.

### EXAMPLE 4

472 g prepared as indicated in example 2 are heated at 40-50 °C and mixed with 500 g of the product obtained in example 3.

### APPLICATION EXAMPLES

### APPLICATION EXAMPLE A

Retanning and fatliquoring of wet blue cow leathers, thickness: 1,5-1,6 mm (percentages are based on the shaved weight).

Wet Blue leathers (half of a leather) are given into a drum and 300 % of water at 40°C are added, followed by 0.2 % of formic acid and the drum is rotated for 15 minutes. The bath is drained. Then 150 % of water and 2 % of sodium formate and 1 % of sodium bicarbonate arc added and drumming is continued for 60 minutes at 35-40 °C. The pH is increased to 5.0. The bath is drained. 200 % of water at 35°C is added and the goods are washed for 10 minutes, then the bath is drained. 100 % of water at 40 °C, 10 % of the instant retanning and lubricating composition are added and the drum is rotated for 60 minutes at this temperature. 0.5 % of formic acid is added and the drum is rotated for 10 minutes at 40 °C. Other 0.5 % of formic acid is added and the drum is rotated for 20 minutes 40 °C: pH is 3.6.

The bath is drained. 300 % of water at 25°C is added and the goods are washed for 10 minutes, then the bath is drained and leathers are discharged, horsed up and dried with one of the conventionally dry system (samm/sett out/vac dry/Hang dry/condition/stake/air off), staked for assessing the properties of the leathers and the light, heat fastness as well as the fogging.

The leather is retanned and fatliquored very regularly, is firm, tight, soft and is optimally suitable for further processing in the tannery. Light and heat resistances are good, fogging values are excellent.

### APPLICATION EXAMPLE B

Retanning and fatliquoring of wet blue cow leathers, thickness 1.1 - 1.2 mm (percentages are based on the shaved weight).

Wet Blue leathers (half of a leather) are given into a drum and 300 % of water at 40°C are added, followed by 0.2 % of formic acid and the drum is rotated for 20 minutes. The bath is drained. Then 100 % of water, 2 % of a neutralising Syntan (like Tanicor AS 6), 1.5 % of sodium bicarbonate and 3.0 % of the instant composition are added and drumming is continued for 75 minutes at 35 - 40 °C. The bath is drained. 300 % of water at 40°C is added and the goods are washed for 10 minutes, then the bath is drained. 100 % of water at 40 °C, 3 % of the instant retanning and lubricating composition are added and drumming is continued for 20 minutes, 3 % of a polyacrylate 30 % sol (like Tergotan PR) is added and drumming is continued for 20 minutes, 4.0 % of a phenol/cresol synthan (like Sandotan SG powder) and 4.0 % of TARA powder (vegetable tanning agent) are added and drumming is continued for 30 minutes, 3 % of Dye (Melioderm Deep Brown F) is added and drumming is continued for 60 minutes, 0.5 % of formic acid are added and the drum is rotated for 15 minutes at this temperature, 1.0 % of formic acid is added and the drum is rotated for 30 minutes at 35 -40 °C.

The bath is drained. 200 % of water at 60 °C is added and the goods are washed for 10 minutes, then the bath is drained. 150 % of water is added and 8.0 % of the instant retanning and lubricating composition is added and the drum is rotated for 60 minutes at 60 °C. 0.5% of formic acid is added and the drum is rotated.

Then the bath is drained and leathers are discharged, horsed up and dried with one of the conventionally dry systems (samm/sett out/vac dry/Hang dry/condition/stake/air off), staked, for assessing the properties of the leathers

The leather is retanned and fatliquored very regularly, is firm, tight, very soft and is optimally suitable for further processing in the tannery.

### APPLICATION EXAMPLE C

Retanning and fatliquoring of wet blue caw leathers, thickness 1.5 - 1.6 mm (percentages are based on the shaved weight).

Wet Blue leather (half of a leather) are given into a drum and 200 % of water at 30°C are added, followed by 1.0 % of a wetting agent (like Tergolix W 01) and 0.5 % of acetic acid and the drum is rotated for 30 minutes. The bath is drained. Then 50 % of water at 35 °C, 5 % of Baychrom F (Chrom basic sulphate) are added and drumming is continued for 90 minutes at 35 - 40 °C. The leather is left in the bath during the night.

At the morning pH is 3.5. 100 % of water of 7°Bé at 50°C and 1 % of sodium formate are added and the drum is rotated for 30 minutes. pH is 4.8. The bath is drained. 100 % of water of 7°Bé at 35 °C, 1 % of sodium formiate are added and rotated for 20 minutes, 1% of sodium bicarbonate is added and rotated for 40 minutes. pH is 5.6-5.7. The leathers are washed with 300 % of water. The bath is drained. 100 % of water at 40 °C, 20 % of a phenol synthan 50% sol (like Syncotan MRL) are added and drumming for 60 minutes. 1% of formic acid is added and drum is rotated for 20 minutes. The bath is drained.

50 % of water is added at 20 °C, 1% of Dye (Bruno Melioderm G) is added and drum is rotated for 30 minutes. 100 % of water at 50 °C, 10 % of the instant retanning and fatliquoring composition is added and the drum is rotated for 60 minutes. 1% of formic acid is added and the drum is rotated for 20 minutes. The bath is drained.

200 % of water at 15 °C is added and the drum is rotated for 10 minutes. The bath is drained and the leathers are discharged and dried with one of the conventionally dry system (samm/sett out/vac dry/Hang dry/condition/stake/air off), staked, for assessing the properties of the leathers.

The leather is retanned and fatliquored very regularly, is firm, tight, soft and are optimally suitable for further processing in the tannery.

| | | | |
|---|---|---|---|
| **Article:** | Heat & Light Fastness-Fatliquors | **Thickness:** | 1.5mm |
| **Raw Material:** | Wet Blue | **Method:** | Direct |
| **Origin:** | LGR | **Colour:** | **Natural** |
| **Tannage:** | Chrome | **% Based on:** | Shaved Weight |
| **Date:** | | **Trial Number:** | **1201** |

| **Process** | **%** | **Chemicals** | **°C** | | **Min.** | **pH** | **Comments** |
|---|---|---|---|---|---|---|---|
| WASH | 300 | Water | 40 | | | | |
| | 0.2 | Formic Acid | | | 15 | | |
| DRAIN | | | | | | | |
| NEUTRALISE | 150 | Water | 35 | | | | |
| | 2.0 | Sodium Formate | | | | | |
| | 1.0 | Sodium Bicarbonate | | | 60 | 5,0 | Cut: |
| DRAIN | | | | | | | |
| WASH | 200 | | | | 10 | | |
| DRAIN | | | | | | | |
| RETAN | 100 | Water | 40 | | | | |
| | 10.0 | Composition as described above | | | 60 | | |
| + | 0.5 | Formic Acid | | | 10 | | |
| + | 0.5 | Formic Acid | | | 20 | 3,6 | |
| DRAIN | | | | | | | |
| WASH | 300 | Water | 25 | | 10 | | |
| DRAIN | | | | | | | |
| HORSE UP | | | | | | | |
| SAMM/SETT OUT/VAC DRY/HANG DRY/CONDITION/STAKE/AIR OFF | | | | | | | |

| | | | |
|---|---|---|---|
| **Customer:** | Internal | | |
| **Article:** | Upholstery-Automotive | **Thickness:** | 1.1 - 1.2 mm |
| **Raw: Material** | Wet Blue | **Method:** | Direct |
| **Origin:** | LGR | **Colour:** | **Brown** |
| **Tannage:** | Chrome | **% Based on**: | shaved weight |
| **Date:** | 13.07.2006 | Trial **Number:** | **1201** |

| **Process** | **%** | **Chemicals** | **°C** | | **Min**. | **pH** | **Comments** |
|---|---|---|---|---|---|---|---|
| WASH | 300 | Water | 40 | | | | |
| | 0.2 | Formic Acid | | | 20 | | |
| DRAIN | | | | | | | |
| NEUTRALISE | 100 | Water | 40 | | | | |
| | 2.0 | TANICOR AS6 | | | | | |
| + | 1.5 | Sodium Bicarbonate | | | | | |
| + | 3.0 | Composition D as described above | | | 75 | | |
| DRAIN | | | | | | | |
| WASH | 300 | Water | 40 | | 10 | | |
| DRAIN | | | | | | | |
| RETAN | 100 | Water | 40 | | | | |
| | 3.0 | Composition as described above | | | 20 | | |
| + | 3.0 | TERGOTAN PR | | | 20 | | |
| + | 4.0 | SANDOTAN SG Powder | | | | | |
| + | 4.0 | Tara | | | 30 | | |
| + | 3.0 | Sandoderm Deep Brown F | | | 60 | | |
| + | 0.5 | Formic Acid | | | 15 | | |
| + | 1.0 | Formic Acid | | | 30 | | |
| DRAIN | | | | | | | |
| WASH | 200 | Water | 60 | | 10 | | |
| DRAIN | | | | | | | |
| FAT | 150 | Water | 60 | | | | |
| | 8.0 | Composition as described above | | | 60 | | |
| + | 0.5 | Formic Acid | | | 30 | | |
| DRAIN | | | | | | | |
| WASH | 300 | Water | 20 | | 10 | | |
| DRAIN & UNLOAD | | | | | | | |
| SAMM/SET OUT/TOGGLE DRY/CONDITION/STAKE (7+7 twice through machine)/ASSESS/MILL 24 HRS/ ASSESS | | | | | | | |

## Claims

1. A composition comprising the components (A), (B) and (C) wherein
(A) is a reaction product of an ethylenically unsaturated C₄-C₈-dicarboxylic anhydride with C₃-C₄₀-alpha-olefins followed by partial or total neutralisation with a base, in aqueous dispersion with or without solvents,
(B) is a reaction product of ethylenically unsaturated C₄-C₈-dicarboxylic anhydrides with C₁₀-C₄₀-fatty acids or C₄-C₃₀ polycarboxylic acids or C₁₀-C₄₀ fatty alcohols or oxo-alcohols or glycols or polyglycols or C₃-C₂₀ organic amines all being saturated or unsaturated, linear or branched and the fatty acids being ethoxylated and/or propoxylated or having been reacted with polyglycols or glycols, and the polycarboxylic acids being ethoxylated and/or propoxylated or having been reacted with polyglycols or glycols at least with one carboxylic group, whereas the fatty alcohols or oxo-alcohols and the fatty amines can optionally be ethoxylated and/or propoxylated,
and
(C) is a reaction product of (B) with bisulphite or metabisulphite or sulphite or sulphuric acid or oleum, followed by partial or total neutralization with a base where the base is an alkali or earth alkali hydroxide, ammonia or an organic amine in aqueous dispersion with or without solvents.

2. Composition according to claim 1 wherein
in the component (A) a part of the anhydride groups are reacted with alcohols, polyalcohols, glycols or organic amines, or ammonia
in the component (B) the fatty alcohols or oxo-alcohols and the fatty amines have been ethoxylated and/or propoxylated, and the glycols or polyglycols have been reacted with other carboxylic acids or C₄-C₃₀ polycarboxylic acids or derivates of carboxylic or polycarboxylic acids.

3. Composition according to claim 1 or 2 wherein
in the component (A) the dicarboxylic anhydride is maleic anhydride and the alpha-olefins have a chain length of 12 to 30 C-atoms and the base is ammonia, an amine or an alkali or earth alkali hydroxide in aqueous dispersion with or without solvents,
in the component (B) the dicarboxylic anhydride is maleic anhydride, and the fatty acids or fatty alcohols or oxo-alcohols have a chain length of 12 to 30 C-atoms and are ethoxylated/propoxylated with 2- 25 mol of EO/ PO or the fatty acids are reacted with polyglycols 100 - 1200, and
the component (C) is a reaction product of (B) with sodium bisulphite carried out in aqueous medium.

4. Composition according to claim 3 wherein
in the component (A) the alpha-olefins have a chain length of 18 to 24 C-atoms and the base is NaOH,
in the component (B) the fatty acids or fatty alcohols or oxo-alcohols have a chain length of 12 to 20 C-atoms and have one or more double bonds, and the fatty acids and fatty alcohols or oxo-alcohols have been ethoxylated.

5. Composition according to claim 4 wherein
in the component (B) the fatty acids have been reacted prior to the reaction with maleic anhydride with polyethylene glycols or glycols.

6. Composition according to claim 3 or 4 wherein
in the component (A) the alpha-olefins have a chain length of 20 to 22 C-atoms,
in the component (B) the fatty acid is oleic acid and wherein the polyethylene glycol is a polyethylene glycol of the formula HO(CH₂CH₂O)ₙH with an average number of n from 2 to 25.

7. Composition according to any of the preceding claims wherein the molar ratio of (A):[(B) + (C)] is from 5:100 to 100:5 and the molar ratio from (B):(C) is from 5:100 to 100:5.

8. Composition according to claim 7 wherein the molar ratio of (A):[(B)+(C)] is from 50:100 to 100:50, and the molar ratio from (B):(C) is from 20:100 to 100:20.

9. Composition according to any of the preceding claims, further comprising amides and esters of the component (A).

10. Composition according to any of the preceding claims, further comprising at least one formulation additive (S) selected from
• water or an organic solvent or mixture and/or solubiliser or mixture miscible with or soluble in (A) and (B) and (C) or in which (A) and (B) and (C) are soluble,
• a defoamer,
• a natural or mineral oil,
• a surfactant,
• a lecithine and
• a biocide.

11. Process for producing a composition according to claim 1 by mixing the components (A), (B) and (C) and optionally adding any formulation additive (S).

12. Use of a composition according to claims 1 to 10 for retanning and fatliquoring of pelts, skins, hides, leather intermediate products or non-finished leather.

13. A process for retanning or fatliquoring of pelts, skins, hides, leather intermediate products or non-finished leather comprising a treatment with a composition according to any of claims 1 to 10.

## Patentansprüche

1. Zusammensetzung, umfassend die Bestandteile (A), (B) und (C), wobei
(A) ein Produkt der Umsetzung eines ethylenisch ungesättigten C₄-C₈-Dicarbonsäureanhydrids mit C₃-C₄₀-alpha-Olefinen mit anschließender teilweiser oder vollständiger Neutralisierung mit einer Base ist, in einer wässrigen Dispersion mit oder ohne Lösemittel,
(B) ein Produkt der Umsetzung von ethylenisch ungesättigten C₄-C₈-Dicarbonsäureanhydriden mit C₁₀-C₄₀-Fettsäuren oder C₄-C₃₀-Polycarbonsäuren oder C₁₀-C₄₀-Fettalkoholen oder Oxoalkholen oder Glykolen oder Polyglykolen oder C₃-C₂₀ organischen Aminen ist, wobei alle diese gesättigt oder ungesättigt, geradkettig oder verzweigt sein können und die Fettsäuren ethoxyliert und/oder propoxyliert sind oder mit Polyglykolen oder Glykolen umgesetzt wurden, und wobei die Polycarbonsäuren ethoxyliert und/oder propoxyliert sind oder mit Polyglykolen oder Glykolen umgesetzt wurden, was zumindest eine ihrer Carbonsäuregruppen betrifft, während die Fettalkohole oder Oxoalkohole und die Fettamine möglicherweise ethoxyliert und/oder propoxyliert sein können, und
(C) ein Produkt der Reaktion von (B) mit Bisulfit oder Metabisulfit oder Sulfit oder Schwefelsäure oder rauchender Schwefelsäure ist, welches anschließend mit einer Base teilweise oder vollständig neutralisiert wird, wobei es sich bei der Base um ein Alkali- oder Erdalkalihydroxid, Ammoniak oder ein organisches Amin in wässriger Dispersion mit oder ohne Lösemittel handelt.

2. Zusammensetzung gemäß Anspruch 1, wobei
im Bestandteil (A) ein Teil der Anhydridgruppen mit Alkoholen, Polyalkoholen, Glykolen oder organischen Aminen oder Ammoniak umgesetzt wird
im Bestandteil (B) die Fettalkohole oder Oxoalkohole und die Fettamin ethoxyliert und/oder propoxyliert wurden, und die Glykole oder Polyglykole mit weiteren Carbonsäuren oder C₄-C₃₀-Polycarbonsäuren oder Derivaten von Carbon- oder Polycarbonsäuren umgesetzt wurden.

3. Zusammensetzung gemäß Anspruch 1 oder 2, wobei
im Bestandteil (A) das Dicarbonsäureanhydrid gleich Maleinsäureanhydrid ist und die alpha-Olefine eine Kettenlänge von 12 bis 30 C-Atomen aufweisen und es sich bei der Base um Ammoniak, ein Amin oder ein Alkali- oder Erdalkalihydroxid in wässriger Dispersion mit oder ohne Lösemittel handelt,
im Bestandteil (B) das Dicarbonsäureanhydrid gleich Maleinsäureanhydrid ist, und die Fettsäuren oder Fettalkohole oder Oxoalkohole eine Kettenlänge von 12 bis 30 C-Atomen aufweisen, wobei sie mit 2 bis 25 Mol an EO/PO ethoxyliert/propoxyliert sind, oder die Fettsäuren mit Polyglykolen 100 - 1200 umgesetzt werden, und
der Bestandteil (C) ein Produkt der Umsetzung von (B) mit Natriumbisulfit ist, wobei diese im wässrigen Milieu durchgeführt wird.

4. Zusammensetzung gemäß Anspruch 3, wobei
im Bestandteil (A) die alpha-Olefine eine Kettenlänge von 18 bis 24 C-Atomen aufweisen und die Base gleich NaOH ist,
Im Bestandteil (B) die Fettsäuren oder Fettalkohole oder Oxoalkohole eine Kettenlänge von 12 bis 20 C-Atomen aufweisen und eine oder mehrere Doppelbindungen haben, und die Fettsäuren und Fettalkohole oder Oxoalkohole ethoxyliert wurden.

5. Zusammensetzung gemäß Anspruch 4, wobei
im Bestandteil (B) die Fettsäuren, im Vorfeld der Reaktion mit Maleinsäureanhydrid, mit Polyethylenglykolen oder Glykolen umgesetzt wurden.

6. Zusammensetzung gemäß Anspruch 3 oder 4, wobei
im Bestandteil (A) die alpha-Olefine eine Kettenlänge von 20 bis 22 C-Atomen haben,
im Bestandteil (B) die Fettsäure gleich Ölsäure ist, und wobei das Polyethylenglykol ein Polyethylenglykol mit der Formel HO(CH₂CH₂O)ₙH ist, dessen Anzahl an n im Durchschnitt 2 bis 25 beträgt.

7. Zusammensetzung gemäß einem beliebigen der vorhergehenden Ansprüche, wobei das Molverhältnis von (A):[(B)+(C)] im Bereich von 5:100 bis 100:5 liegt und das Molverhältnis von (B):(C) im Bereich von 5:100 bis 100:5 liegt.

8. Zusammensetzung gemäß Anspruch 7, wobei das Molverhältnis von (A):[(B)+(C)] im Bereich von 50:100 bis 100:50 liegt und das Molverhältnis von (B):(C) im Bereich von 20:100 bis 100:20 liegt.

9. Zusammensetzung gemäß einem beliebigen der vorhergehenden Ansprüche, die weiterhin Amide und Ester des Bestandteils (A) umfasst.

10. Zusammensetzung gemäß einem beliebigen der vorhergehenden Ansprüche, die weiterhin mindestens einen Formulierungshilfsstoff (S) umfasst, welcher aus den folgenden ausgewählt ist
• Wasser oder einem organischen Lösemittel oder Mischung und/oder Löslichkeitsvermittler oder Mischung, welches/welche mit (A) und (B) und (C) mischbar oder darin löslich ist, oder in welchem (A) und (B) und (C) löslich sind,
• einem Schaumverhüter,
• einem natürlichen oder mineralischen Öl,
• einem Tensid,
• einem Lecithin und
• einem Biozid.

11. Verfahren zur Herstellung einer Zusammensetzung gemäß Anspruch 1, indem die Bestandteile (A), (B) und (C) vermischt werden und möglicherweise ein beliebiger Formulierungshilfsstoff (S) zugesetzt wird.

12. Verwendung einer Zusammensetzung gemäß den Ansprüchen 1 bis 10 zum Nachgerben und Fetten von Pelzen, Häuten, Fellen, Lederzwischenprodukten oder unveredeltem Leder.

13. Verfahren zum Nachgerben oder Fetten von Pelzen, Häuten, Fellen, Lederzwischenprodukten oder unveredeltem Leder, welches eine Behandlung mit einer Zusammensetzung gemäß einem beliebigen der Ansprüche 1 bis 10 umfasst.

## Revendications

1. Composition comprenant les composants (A), (B) et (C) dans laquelle
(A) est un produit de réaction d'un anhydride dicarboxylique en C₄-C₈ à insaturation éthylénique avec des alpha-oléfines en C₃-C₄₀ suivie d'une neutralisation partielle ou totale avec une base, en dispersion aqueuse avec ou sans solvants,
(B) est un produit de réaction d'anhydrides dicarboxyliques en C₄-C₈ à insaturation éthylénique avec des acides gras en C₁₀-C₄₀ ou des acides polycarboxyliques en C₄-C₃₀ ou des alcools gras en C₁₀-C₄₀ ou des oxo-alcools ou des glycols ou des polyglycols ou des amines organiques en C₃-C₂₀, tous étant saturés ou insaturés, linéaires ou ramifiés et les acides gras étant éthoxylés et/ou propoxylés ou ayant été amenés à réagir avec des polyglycols ou des glycols et les acides polycarboxyliques étant éthoxylés et/ou propoxylés ou ayant été amenés à réagir avec des polyglycols ou des glycols au moins avec un groupe carboxylique et les alcools gras ou oxo-alcools et les amines grasses pouvant facultativement être éthoxylés et/ou propoxylés,
(C) est un produit de réaction de (B) avec un bisulfite ou un métabisulfite ou un sulfite ou de l'acide sulfurique ou de l'oléum, suivie d'une neutralisation partielle ou totale avec une base, la base étant un hydroxyde de métal alcalin ou alcalinoterreux, l'ammoniac ou une amine organique en dispersion aqueuse avec ou sans solvants.

2. Composition selon la revendication 1 dans laquelle
dans le composant (A) une partie des groupes anhydrides sont amenés à réagir avec des alcools, des polyols, des glycols ou des amines organique ou de l'ammoniac et
dans le composant (B) les alcools gras ou oxo-alcools et les amines grasses ont été éthoxylés et/ou propoxylés et les glycols ou polyglycols ont été amenés à réagir avec d'autres acides carboxyliques ou des acides polycarboxyliques en C₄-C₃₀ ou des dérivés d'acides carboxyliques ou polycarboxyliques.

3. Composition selon la revendication 1 ou 2 dans laquelle
dans le composant (A) l'anhydride dicarboxylique est l'anhydride maléique et les alpha-oléfines ont une longueur de chaîne de 12 à 30 atomes de carbone et la base est l'ammoniac, une amine ou un hydroxyde de métal alcalin ou alcalinoterreux en dispersion aqueuse avec ou sans solvants,
dans le composant (B) l'anhydride dicarboxylique est l'anhydride maléique et les acides gras ou alcools gras ou oxo-alcools ont une longueur de chaîne de 12 à 30 atomes de carbone et sont éthoxylés/propoxylés avec 2-25 mol d'OE/OP ou les acides gras sont amenés à réagir avec des polyglycols 100-1200 et
le composant (C) est un produit de réaction de (B) avec du bisulfite de sodium effectuée en milieu aqueux.

4. Composition selon la revendication 3 dans laquelle
dans le composant (A) les alpha-oléfines ont une longueur de chaîne de 18 à 24 atomes de carbone et la base est NaOH,
dans le composant (B) les acides gras ou alcools gras ou oxo-alcools ont une longueur de chaîne de 12 à 20 atomes de carbone et une ou plusieurs doubles liaisons et les acides gras et alcools gras ou oxo-alcools ont été éthoxylés.

5. Composition selon la revendication 4 dans laquelle
dans le composant (B) les acides gras ont été amenés à réagir avant la réaction avec de l'anhydride maléique avec des polyéthylèneglycols ou des glycols.

6. Composition selon la revendication 3 ou 4 dans laquelle
dans le composant (A) les alpha-oléfines ont une longueur de chaîne de 20 à 22 atomes de carbone,
dans le composant (B) l'acide gras est l'acide oléique, le polyéthylèneglycol étant un polyéthylèneglycol représenté par la formule HO(CH₂CH₂O)ₙH ayant un nombre moyen n de 2 à 25.

7. Composition selon l'une quelconque des revendications précédentes dans laquelle le rapport molaire de (A):[(B) + (C)] est de 5:100 à 100:5 et le rapport molaire de (B):(C) est de 5:100 à 100:5.

8. Composition selon la revendication 7 dans laquelle le rapport molaire de (A):[(B) + (C)] est de 50:100 à 100:50 et le rapport molaire de (B):(C) est de 20:100 à 100:20.

9. Composition selon l'une quelconque des revendications précédentes, comprenant en outre des amides et des esters du composant (A).

10. Composition selon l'une quelconque des revendications précédentes, comprenant en outre au moins un additif de formulation (S) choisi parmi
- l'eau ou un solvant organique ou un mélange et/ou un agent solubilisant ou un mélange miscibles avec (A) et (B) et (C) ou solubles dans (A) et (B) et (C) ou dans lesquels (A) et (B) et (C) sont solubles,
- un antimousse,
- une huile naturelle ou minérale,
- un tensioactif,
- une lécithine et
- un biocide.

11. Procédé pour la production d'une composition selon la revendication 1 par mélange des composants (A), (B) et (C) et facultativement ajout de tout additif de formulation (S).

12. Utilisation d'une composition selon les revendications 1 à 10 pour le retannage et la nourriture en bain de cuirs en tripe, de peaux, de cuirs bruts, de produits intermédiaires du cuir ou de cuir non fini.

13. Procédé pour le retannage ou la nourriture en bain de cuirs en tripe, de peaux, de cuirs bruts, de produits intermédiaires du cuir ou de cuir non fini comprenant un traitement avec une composition selon l'une quelconque des revendications 1 à 10.
